

# United States Patent Office

2,737,452

Patented Mar. 6, 1956

2,737,452

## STABILIZED FUEL OILS

Willard E. Catlin, Wilmington, and Gordon Bradbury Robbins, Claymont, Del., assignors to E. I. du Pont de Nemours & Company, Wilmington, Del., a corporation of Delaware

No Drawing. Application April 7, 1952,  
Serial No. 281,047

11 Claims. (Cl. 44—62)

This invention relates to stabilized fuel oils and, more particularly, to fuel oils adapted to withstand without deterioration the prolonged oxidizing conditions of storage. This application is a continuation-in-part of applicants' copending application Serial No. 214,855, filed March 9, 1951, and abandoned April 12, 1952.

Fuel oils, that is, hydrocarbon oils boiling above the gasoline range and used as burner and furnace oils and diesel fuels and the like, are produced not only from straight run petroleum hydrocarbon distillates but, also, by thermocracking and catalytic cracking. Until recently, most fuel oils have been straight run but catalytic cracking is fast becoming the most popular method for supplying the increased demand for fuel oils.

Fuel oil blends containing substantial proportions of catalytic cracked stocks, e. g., from approximately 20% to 60% by weight of the blend, with straight run fuel oils are now being marketed. It would be preferable to increase the proportion of catalytic cracked oil or sell catalytic cracked oil exclusively for fuel purposes but this has not been practical because of a serious storage stability problem.

Fuel oils are frequently prone to deterioration on storage and catalytic cracked fuel oil in particular is frequently very unstable and deteriorates badly in storage. The deterioration resulting from the mild but prolonged oxidizing conditions of storage results not only generally in discoloration but in the formation of sludge or sediment which, if not removed, plugs filter screens, orifices, and other parts of the equipment used in burning such fuel. The high susceptibility to deterioration of many catalytic cracked fuel oils has made it necessary to blend them off with larger proportions of the less plentiful but more stable straight run stocks to meet even the minimum stability requirements. Nevertheless, difficulty has been experienced with such fuels and refiners are frequently forced to take back from the distributors oil with considerable oil insoluble residue.

The problem of stabilizing catalytic cracked fuel oils is relatively new. Because of its importance there is a great deal of activity in the field of additives to stabilize fuel oils, but no really satisfactory solution to the problem has been devised. Another approach to the problem has been to develop refining techniques or treating processes to remove the unstable components of catalytic cracked fuel oil to improve its storage stability. Some refiners have been able to achieve quality improvements by certain treating methods, such as acid washing of the oil, but these methods are too costly for commercial application and do not seem to present a solution to the problem. Also, while catalytic cracked fuel oils are the worst performers in the matter of deterioration during storage, the problem does exist to greater or lesser degree with fuel oils generally.

An object of the present invention is to provide an improved stabilized fuel oil. A further object is to provide a stabilized fuel oil containing at least a substantial proportion of catalytic cracked oil. A still further and

more specific object is to provide a stabilized catalytic cracked fuel oil which may be stored without deterioration. Other objects will be apparent from the description of the invention given hereinafter.

The above objects are accomplished according to the present invention by incorporating in a fuel oil a small proportion, at least 0.001% by weight of the fuel oil, of an oil-soluble, basic amino nitrogen-containing addition-type polymer of a plurality of polymerizable ethylenically unsaturated compounds, at least one of which is amine-free and contains from 8 to about 18 carbon atoms in an aliphatic hydrocarbon chain which in the polymer is not part of the main polymer chain preferably predominantly straight chain in nature, and one of which as it exists in the polymer contains a basic amino nitrogen in the side chain, said polymer containing 0.1% to 3.5%, by weight thereof, of basic amino nitrogen.

The optimum proportion of polymer in the fuel oil will be determined by its inherent viscosity, which can be within the range of 0.1 to 3.0 as determined at 0.1% weight/volume concentration in benzene at 25° C. From a practical point of view, 0.001% to 0.1% of the polymer additive having an inherent viscosity between about 0.2 and 1.0, normally will be found to give optimum results:

Although the mechanism by which the fuel oil compositions of this invention operate is not known, experimental work both in laboratory and practical tests has established certain basic requirements for the addition-type polymers as regards composition, structure, and physical properties. For example, it is essential that at least one of the monomeric components employed in making the polymer should introduce an oil-solubilizing or oleophilic structure to insure that the polymer is soluble to the extent of at least 0.001% by weight in various types of fuel oils. In addition, the presence of basic amino groups, either primary, secondary, or tertiary, is necessary to impart the unique sludge inhibiting and dispersing properties which characterize these polymers. The proportion of basic amino nitrogen is best expressed in weight percent based on the total copolymer, and should be within the range of 0.1% to 3.5%. Introduction of the basic amino nitrogen structure can be accomplished by the use of at least one monomeric component containing the amino group or by use of a monomer containing a group which is reactive, when present in the polymer, toward ammonia, or primary or secondary nonaromatic amines. These monomers can also contain oleophilic structures that will assist in contributing to the requisite oil solubility. In addition, some of the polymers coming within the scope of this invention can, without sacrificing either fuel oil solubility or sludge inhibiting and dispersing properties, include certain proportions of monomers that do not themselves yield oil-soluble polymers.

Copolymers useful in the practice of the invention can be prepared by conventional bulk, solution, or dispersion polymerization methods involving known initiators, including oxygen-yielding compounds, such as benzoyl peroxide, and azo compounds, such as alpha, alpha'-azodiisobutyronitrile. Convenient solvents are high-boiling hydrocarbons, particularly those similar to the hydrocarbons in which the copolymers are to be used, such as kerosene. The polymerization processes usually are carried out in an inert atmosphere, e. g., nitrogen or carbon dioxide, at temperatures ranging from 30° C. to 150° C., depending on the catalyst used, and generally at temperatures between 50° C. and 70° C. when alpha, alpha'-azodiisobutyronitrile is used as the catalyst. It is important to carry the copolymerization substantially to completeness so that no unpolymerized monomers remain and the pro-

portions of each component in the final product are essentially those of the original monomer mixture.

The following examples wherein all parts are by weight unless otherwise stated, illustrate typical polymers adapted for use in the present invention.

#### EXAMPLE I

47.5 parts of n-octyl methacrylate, 2.5 parts of beta-diethylaminoethyl methacrylate, and 0.25 part of alpha,alpha'-azodiisobutyronitrile were heated together in a polymerization reactor under an atmosphere of oxygen-free nitrogen at  $58 \pm 3^\circ$  C. for 18 hours, stirring being effected by bubbling a stream of nitrogen through the polymerization mixture. There was thus obtained a fuel oil-soluble, tacky, resinous copolymer of the two polymerizable components in essentially the proportions charged, i. e., 95/5.

#### EXAMPLE II

1020 parts of technical lauryl methacrylate, 100 parts of methacrylanilide, 60 parts of beta-diethylaminoethyl methacrylate, 300 parts of mineral oil and 3.6 parts of alpha,alpha'-azodiisobutyronitrile were agitated together at  $60 \pm 2^\circ$  C. under nitrogen. After two hours some thickening of the charge was observed and during the next 16 hours, 900 parts more of mineral oil was added gradually as the polymerization proceeded. There was thus obtained a barely stirrable fuel oil solution of a copolymer of the three polymerizable components in essentially the proportions charged, i. e., 86.4/8.5/5.1. Similar results were obtained when kerosene was used in place of mineral oil.

The technical lauryl methacrylate used in the preparation above is the methacrylic acid ester of technical lauryl alcohol which is obtained by reduction of the fatty acids of coconut oil and is a mixture of saturated straight chain alcohols ranging from about 10 to 18 carbon atoms. A typical example will contain approximately 3% C<sub>10</sub>, 61% C<sub>12</sub>, 23% C<sub>14</sub>, 11% C<sub>16</sub> and 2% C<sub>18</sub> alcohols.

#### EXAMPLE III

170 parts of technical lauryl methacrylate, 20 parts of methacrylanilide (N-phenylmethacrylamide), 10 parts of glycidyl methacrylate and 1.2 parts of alpha,alpha'-azodiisobutyronitrile were heated together in a polymerization reactor for 8 hours at  $65^\circ$  C., as in Example I. The 85/10/5 lauryl methacrylate/methacrylanilide/glycidyl methacrylate copolymer thus obtained was removed from the polymerization reactor and thoroughly mixed with twenty-two parts of technical diamylamine (2 molar proportions based on the copolymer) by careful milling on a two-roll rubber mill. The resultant mixture was placed in a closed container and warmed for 24 hours at about  $60^\circ$  C. to complete the reaction of the amine with the epoxide structures in the polymer. This reaction involves scission of the oxirane rings in the glycidyl methacrylate units by the diamylamine to give units containing gamma-diamylamino-beta-hydroxypropyl radicals as more fully disclosed in application Serial No. 176,918, filed July 31, 1950, now abandoned, in the name of M. E. Cuper, assigned to the assignee of this application. The final product is thus a lauryl methacrylate/methacrylanilide/gamma-diamylamino - beta - hydroxypropyl methacrylate copolymer.

#### EXAMPLE IV

90 parts of technical lauryl methacrylate and 10 parts of glycidyl methacrylate were copolymerized as in Example II by heating at  $60^\circ$  C. for 24 hours in solution in 100 parts of highly refined petroleum white oil in the presence of 0.6 part of alpha,alpha'-azodiisobutyronitrile.

To the oil solution of the copolymer thus obtained there was then added 9.4 parts of technical diamylamine (0.85 molar proportion based on the copolymer) and the mixture was heated to  $80^\circ$  C. for about 1 hour to effect reaction of the diamylamine with the oxirane rings in the glycidyl methacrylate units in the copolymer in the manner explained in Example III, to obtain a white oil solution of a lauryl methacrylate/glycidyl methacrylate/gamma-diamylamino-beta-hydroxypropyl methacrylate copolymer.

#### EXAMPLE V

A mixture of 19 parts of vinyl laurate, 1 part of allyl glycidyl ether and 0.12 part of alpha,alpha'-azodiisobutyronitrile was heated for 6 hours at  $65^\circ$  C. as in Example III. To the resulting 95/5 vinyl laurate/allyl glycidyl ether copolymer was added 1.1 parts of technical diamylamine and the reaction mixture allowed to stand for several days at room temperature. There was thus obtained a fuel oil-soluble vinyl laurate/allyl glycidyl ether/allyl gamma - diamylamino - beta - hydroxypropyl ether copolymer.

#### EXAMPLE VI

25 A pressure-resistant reaction vessel was charged with 20 parts of beta-diethylaminoethyl methacrylate, 50 parts of 2-ethylhexyl acrylate and 0.5 part of alpha,alpha'-azodiisobutyronitrile. The vessel was closed, flushed with nitrogen and evacuated, pressurized with isobutylene under 3000 atmospheres pressure, and heated with agitation for 4 hours at about  $65^\circ$  C. The reactor was then cooled, vented to the atmosphere and the resinous product removed. There was thus obtained a 69/16.4/14.6 2-ethylhexyl acrylate/beta-diethylaminoethyl methacrylate/isobutylene copolymer as a fuel oil-soluble, viscous, tacky resin.

Another copolymerization reaction was carried out as above, with 40 parts of lauryl methacrylate, 10 parts of beta-dimethylaminoethyl methacrylate, 50 parts of benzene, 0.5 part of alpha,alpha'-azodiisobutyronitrile and ethylene under 1000 atmospheres pressure. There was thus obtained a 64/18/18 lauryl methacrylate/beta-dimethyl/aminoethyl methacrylate/ethylene copolymer as a fuel oil-soluble, viscous, tacky resin.

45

#### EXAMPLE VII

80 parts of sec-capryl methacrylate (B. P. 70-72° C./0.5-0.7 mm. of mercury), prepared by ester interchange of sec-capryl alcohol with methyl methacrylate in the presence of tetraisopropyl titanate as catalyst (as was fully disclosed in application Serial No. 256,373, filed November 14, 1951, in the name of J. H. Haslam and assigned to the assignee of the present application), 50 parts of beta-diethylaminoethyl methacrylate and 0.5 part of alpha,alpha'-azodiisobutyronitrile were heated together for 5 hours at  $65^\circ$  C. in the manner of Example III above. There was thus obtained an 80/20 sec-capryl methacrylate/beta-diethylaminoethyl methacrylate copolymer as a fuel oil-soluble, soft, sticky, rubbery resin.

#### EXAMPLE VIII

100 parts of tridecyl methacrylate from a commercially available, branched-chain primary tridecyl alcohol, 40 parts of beta-diethylaminoethyl methacrylate, 60 parts of styrene and 1 part of alpha,alpha'-azodiisobutyronitrile were heated for 20 hours at  $65^\circ$  C. in the manner of Example III. There was thus obtained a 50/20/30 tridecyl methacrylate/beta-diethylaminoethyl methacrylate/styrene copolymer as a fuel oil-soluble, rather stiff, rubbery resin.

#### EXAMPLE IX

75 A mixture of 180 parts of lauryl methacrylate, 14.5

parts of N-(beta-vinyloxyethylformamide) (B. P. 87° C./0.9 mm. mercury, prepared by the aminolysis of methyl formate with beta-vinyloxyethyl amine as disclosed in application Serial No. 269,339, filed January 31, 1952, now abandoned, in the name of John C. Sauer and assigned to the assignee of the present application), and 1 part of alpha,alpha'-azodiisobutyronitrile was heated for 4 hours at 65° C. in the manner of Example III. There was thus obtained a lauryl methacrylate/N-(beta-vinyloxyethyl)formamide copolymer as a fuel oil-soluble, clear, tacky, rubber-like resin. 10

## EXAMPLE IX-A

To a solution of 90 parts of the above lauryl methacrylate/N-(beta-vinyloxyethyl)formamide copolymer in about 400 parts of benzene was added 110 parts of 18% aqueous hydrochloric acid, and the resulting mixture heated at a gentle reflux for one hour with stirring. The resulting creamy emulsion was treated with an excess of 20% aqueous sodium hydroxide solution and the organic layer thereby obtained removed, washed well with water and any retained benzene-water removed by evaporation at steam bath temperatures under atmospheric pressure and finally under reduced pressure. There was thus obtained a fuel oil-soluble, highly viscous, tacky copolymer which upon analysis was found to contain 0.25% primary amino nitrogen, indicating the presence of 1.4% combined beta-vinyloxyethyl amine groups. 20 30

## EXAMPLE X

A branched chain ar-dodecylstyrene was prepared by acetylation of a commercial mixture of detergent intermediate type, branched chain dodecylbenzenes with acetyl chloride in the presence of aluminum chloride, selective catalytic hydrogenation of the resulting ketone with nickel catalyst, and dehydration of the carbinol by refluxing with xylene containing iodine. 9 parts of the ar-dodecylstyrene fraction (B. P. 135-140° C./4 mm. of mercury), 1 part of beta-diethylaminoethyl methacrylate and 0.07 part of alpha,alpha'-azodiisobutyronitrile were heated for 5 hours at 65° C. There was obtained a 90/10 ar-dodecylstyrene/beta-diethylaminoethyl methacrylate copolymer as a fuel oil-soluble, high viscous product, tacky at room temperature. 40 45

The polymer additives used in preparing the fuel oil compositions of this invention can be incorporated in the fuel oils by simply blending with stirring at ordinary temperature or, if desired, a mixture of the fuel oil and the additive polymer or polymers can be heated to elevated temperatures, e. g., 100-130° C. with agitation. 50

In the tables given hereinafter showing the results of subjecting fuel oil compositions of the present invention to various tests, all proportions are by weight unless otherwise stated. 55

An accelerated storage test was carried out on samples of catalytic cracked fuel oil #2 distillate inhibited by incorporating therein small amounts of various polymers. In this particular test, 10 cc. portions of the treated fuel oil contained in 20 cc. clear glass vented vials were exposed to indirect sunlight at room temperature. The samples were observed daily and the number of days required for the first appearance of haze and cloudiness in the oil represent the appearance of oil-insoluble products which is the first indication of sludge and precipitate formation in the oil. In some instances, the first appearance of sediment was also noted, this usually occurring somewhat later. The results of this accelerated storage test are given in Tables I to VI below with respect to various copolymers in various concentrations except for Table III-A where a modified test as explained in connection with that table, was used. 60 65 70 75

Table I

## METHACRYLATES AND ACRYLATES OF VARIOUS ALCOHOLS

| Added Copolymer                                                   | Concen-<br>tration,<br>percent | Days to first appearance of |                            |     |     |
|-------------------------------------------------------------------|--------------------------------|-----------------------------|----------------------------|-----|-----|
|                                                                   |                                | Haze<br>(control)           | Sedi-<br>ment<br>(control) |     |     |
| 1. n-Octyl methacrylate/diethylaminoethyl methacrylate 80/20      | 0.006                          | 7                           | (2)                        |     |     |
| 2. Decyl methacrylate/diethylaminoethyl methacrylate 80/20        | 0.005                          | >15                         | (5)                        | >23 | (6) |
| 3. Sec. Capryl methacrylate/diethylaminoethyl methacrylate 80/20  | 0.005                          | >15                         | (5)                        | >23 | (6) |
| 4. 2-ethylhexylacrylate/diethylaminoethyl methacrylate 80/20      | 0.12                           | 3                           | (1)                        |     |     |
| 5. Lauryl methacrylate/diethylaminoethyl methacrylate 80/20       | 0.005                          | >15                         | (5)                        | >23 | (6) |
| 6. Tridecyl methacrylate/dimethylaminoethyl methacrylate 75/25    | 0.006                          | 7                           | (1)                        |     |     |
| 7. Cetyl methacrylate/dimethylaminoethyl methacrylate 75/25       | 0.006                          | 8                           | (1)                        |     |     |
| 8. Octadecyl methacrylate/dimethylaminoethyl methacrylate 75/25   | 0.006                          | 7                           | (1)                        |     |     |
| 9. Octadecenyl methacrylate/diethylaminoethyl methacrylate 83/17  | 0.005                          | 8                           | (5)                        | >23 | (6) |
| 10. Octylphenyl methacrylate/diethylaminoethyl methacrylate 90/10 | 0.05                           | 6                           | (4)                        | >7  | (6) |
| 11. n-Butylmethacrylate/diethylaminoethyl methacrylate 80/20      | 0.006                          | 2                           | (2)                        |     |     |

Copolymer #11, which does not fall within the scope of the invention, illustrates that copolymers without side chains containing at least eight carbon atoms, show no appreciable inhibiting action in this test.

Table II

## VARIATION IN COPOLYMER CONCENTRATION

| Added Copolymer                                                    | Concen-<br>tration,<br>percent | Days to first<br>appearance of |                            |
|--------------------------------------------------------------------|--------------------------------|--------------------------------|----------------------------|
|                                                                    |                                | Haze<br>(control)              | Sedi-<br>ment<br>(control) |
| Technical lauryl methacrylate/diethylaminoethyl methacrylate 80/20 | 0.12                           | >13                            | (1)                        |
|                                                                    | 0.006                          | 12                             |                            |
|                                                                    | 0.003                          | 8                              |                            |
|                                                                    | 0.0015                         | 5                              |                            |

Table III

## VARIATION IN RATIO OF POLYMER COMPONENTS AND IN COPOLYMER CONCENTRATION

| Ratio Lauryl methacrylate/diethylaminoethyl methacrylate | Concen-<br>tration,<br>percent | Days to first<br>appearance of |               |
|----------------------------------------------------------|--------------------------------|--------------------------------|---------------|
|                                                          |                                | Haze                           | Sedi-<br>ment |
| 1. Control                                               |                                | 4                              | 7             |
| 2. 99/1                                                  | 0.010                          | 4                              | 12            |
|                                                          | 0.100                          | 5                              | >19           |
| 3. 97.5/2.5                                              | 0.001                          | 4                              | 12            |
| 4. 95/5                                                  | 0.010                          | 8                              | >19           |
| 5. 90/10                                                 | 0.005                          | 5                              | >17           |
| 6. 80/20                                                 | 0.005                          | 7                              | >17           |
| 7. 70/30                                                 | 0.005                          | 8                              | >17           |
| 8. 25/75                                                 | 0.005                          | 3                              | 5             |
| 9. 10/90                                                 | 0.005                          | 2                              | 2             |

Copolymers #8 and #9 do not embody the invention inasmuch as they contain in excess of 3.5%, by weight, of basic amino nitrogen due to the large proportion of diethylaminoethyl methacrylate, and actually give poorer results than the control.

Table III-A below supplements Table III. The test used here differed from that in Tables I to VI in that the samples were maintained at 110° F. in the dark, the weeks to the first appearance of sediment being observed. The fuel oil used was Sinclair 100% fluid catalytically cracked light cycle oil.

Table III-A

| Ratio Lauryl methacrylate/diethylaminoethyl methacrylate | Concentration, percent | Weeks to first appearance of sediment |
|----------------------------------------------------------|------------------------|---------------------------------------|
| 1. Control                                               |                        | 3                                     |
| 2. 100/0                                                 | .005                   | 2                                     |
| 3. 95/5                                                  | .005                   | 5                                     |
| 4. 90/10                                                 | .005                   | 9                                     |
| 5. 80/20                                                 | .005                   | 12                                    |
| 6. 70/30                                                 | .005                   | 12                                    |
| 7. Control                                               |                        | 6                                     |
| 8. 80/20                                                 | .002                   | 11                                    |
| 9. 70/30                                                 | .002                   | 9                                     |
| 10. 50/50                                                | .002                   | 8                                     |

## 5 VARIATION IN LONG-CHAIN COMPONENT

8 Table V

| Copolymer Ratio                                                    | Concen-<br>tration,<br>percent | Days to first ap-<br>pearance of— |          |
|--------------------------------------------------------------------|--------------------------------|-----------------------------------|----------|
|                                                                    |                                | Haze                              | Sediment |
| 1. Control                                                         |                                | 4                                 | 6        |
| 2. Lauryl fumarate/DB 1/93/7                                       | .005                           | 7                                 | >17      |
| 3. Vinyl laurate/beta-(N,N-dimethylamino) ethyl vinyl ether 90/10  | .005                           | 5                                 | 13       |
| 4. Vinyl laurate/DB 80/20                                          | .0025                          | 5                                 | —        |
| 5. Octylphenyl methacrylate/DB 90/10                               | .005                           | 6                                 | 7        |
| 6. Control                                                         |                                | 5                                 | 6        |
| 7. Vinyl lauryl ether/vinyl diethylamino ethyl ether 80/20         | .05                            | 7                                 | >13      |
| 8. Control                                                         |                                | 4                                 | 6        |
| 9. Cyclohexyl styrene/N-tertiaryoctylaminoethyl methacrylate 67/33 | .05                            | 6                                 | 6        |
| 10. Dodecyl styrene/DB 90/10                                       | .005                           | 7                                 | 13       |
| 11. Octadecyl styrene/4-vinyl pyridine 80/20                       | .005                           | 20                                | 23       |
|                                                                    |                                | 13                                | 14       |

15 DB is diethylaminoethyl methacrylate.

Table VI

## 30 COPOLYMERS WITH THREE COMPONENTS

| Copolymer Ratio                                                           | Concen-<br>tration,<br>percent | Days to first ap-<br>pearance of |          |
|---------------------------------------------------------------------------|--------------------------------|----------------------------------|----------|
|                                                                           |                                | Haze                             | Sediment |
| 1. Control                                                                |                                |                                  | 4        |
| 2. LM 1/Styrene/DB 2:                                                     |                                |                                  |          |
| 60:30:10                                                                  | .005                           |                                  | 17       |
| 45:45:10                                                                  | .005                           |                                  | 6        |
| 50:30:20                                                                  | .005                           |                                  | 8        |
| 40 3. LM/N-tertiaryoctyl-acrylamide/DB:                                   |                                |                                  |          |
| 45:45:10                                                                  | .005                           |                                  | 7        |
| 30:60:10                                                                  | .005                           |                                  | 7        |
| 20:70:10                                                                  | .005                           |                                  | 7        |
| 30:50:20                                                                  | .005                           |                                  | 7        |
| 45 4. LM/Butadiene/DB 17.5:65:17.5                                        | { .05                          |                                  | 7        |
| 5. Control                                                                | .10                            |                                  | 6        |
| 6. LM/methacrylanilide/2-methyl-5-vinylpyr-<br>idine 85/10/5              | 0.012                          |                                  | 27       |
| 7. Decyl acrylate/methacrylanilide/DB 85/7.5/7.5                          | 0.003                          |                                  | 13       |
| 8. LM/methacrylanilide/ <i>p</i> -dimethylamino-<br>methylstyrene 85/10/5 | 0.012                          |                                  | 20       |
| 9. Control                                                                | .006                           |                                  | 1        |
| 10. LM/methacrylanilide/DB 85/15/5                                        | 0.006                          |                                  | 18       |

15 LM is technical lauryl methacrylate.

15 DB is diethylaminoethyl methacrylate.

| Basic Comonomer                                                                            | Ratio      | Concen-<br>tration | Days to first<br>appearance of |          |
|--------------------------------------------------------------------------------------------|------------|--------------------|--------------------------------|----------|
|                                                                                            |            |                    | Haze                           | Sediment |
| 1. Control                                                                                 |            |                    | 4                              | 7        |
| 2. LM/beta-aminoethyl vinyl-<br>ether                                                      | 97:3       | .005               | 6                              | >17      |
| 3. LM/beta-aminoethyl vinyl-<br>ether                                                      | 95:5       | .005               | 6                              | 55       |
| 4. Control                                                                                 |            |                    | 4                              | 5        |
| 5. LM/N-tertiary-octylamino-<br>ethyl methacrylate                                         | 80:20      | .005               | 7                              | >17      |
| 6. LM/alpha-methyl-benzyl-<br>aminoethyl methacrylate                                      | 85:15      | .005               | 5                              | 9        |
| 7. LM/methacrylanilide/vinyl<br>beta-dimethylaminoethyl ether                              | 85:7.5:7.5 | .005               | 5                              | 8        |
| 8. LM/dimethylamino-methyl-<br>styrene                                                     | 95:5       | .005               | 7                              | >23      |
| 9. LM/2,3-dimethyl-3-dimethyl-<br>aminopropyl methacrylate                                 | 90:10      | .005               | 5                              | >26      |
| 10. LM/beta-(N,N-di-2-ethyl-<br>hexylaminoethyl methacrylate                               | 60:40      | .005               | 7                              | >7       |
| 11. LM/Bis(diethylaminoethyl)-<br>malonate                                                 | 90:10      | .005               | 5                              | 7        |
| 12. Control                                                                                | { 97.5:2.5 | .005               | 6                              | >18      |
|                                                                                            | 95:5       | .005               | 6                              | 11       |
| 13. LM/4-vinyl pyridine                                                                    | 90:10      | .005               | 7                              | 11       |
|                                                                                            | 80:20      | .005               | 7                              | 11       |
| 14. Control                                                                                |            |                    | 4                              | —        |
| 15. LM/methacrylanilide/<br>glycidyl methacrylate<br>+diethyl amine (See Ex-<br>ample III) | 85/10/5    | 0.005              | 13                             | —        |
| 16. Control                                                                                |            |                    | 1                              | —        |
| 17. LM/2-methyl-5-vinyl pyrid-<br>ine                                                      | 90:10      | 0.003              | 6                              | —        |
| 18. LM/diisopropylaminoethyl<br>methacrylate                                               | 80:20      | 0.012              | 8                              | —        |

50 Samples of catalytic cracked fuel oil #2 distillate were inhibited by incorporating therein small amounts of technical lauryl methacrylate/diethylaminoethyl methacrylate 80/20 copolymer. The samples were subjected to an accelerated storage test in vented glass bottles at 110° F. for 12 weeks in the dark. The samples were examined weekly for the first appearance of sediment and at the end of the 12 weeks' period the samples were compared in color using the ASTM NPA method and were analyzed for soluble and insoluble residue using the following method. The sample is filtered at room temperature by gravity through #5 filter paper. The container and filter paper are washed with naphtha. The filtrate is analyzed for soluble residue by steam jet evaporation. The insoluble residue formed during the aging test is dissolved from the container and filter paper with a 50-50 mixture of acetone and methanol and determined by air jet evaporation according to ASTM Method D-525-46. Both sol-

uble and insoluble residue are expressed in mg./100 ml. of fuel. The results of the tests are as follows:

Table VII

EFFECT OF TECHNICAL LAURYL METHACRYLATE/ DIETHYLAMINOETHYL METHACRYLATE 80/20 COPOLYMER ON FUEL OILS STORED 12 WEEKS AT 110° F. IN VENTED GLASS BOTTLES IN THE DARK

| Fuel                                     | Additive Conc., Wt. Percent | Soluble Residue, mg./100 ml. | Insoluble Residue, mg./100 ml. | Time to First Appearance of Sediment | NPA Color | 10 |
|------------------------------------------|-----------------------------|------------------------------|--------------------------------|--------------------------------------|-----------|----|
| Low sulfur thermofor catalytic cracked.  | None                        | 11                           | 7                              | 6 weeks                              | 4½        |    |
| Do                                       | 0.01                        | 4                            | 4                              | None at 12 weeks                     | 3 15      |    |
| High sulfur thermofor catalytic cracked. | None                        | 10                           | 7                              | 10 weeks                             | 4         |    |
| Do                                       | 0.01                        | 5                            | 4                              | 12 weeks                             | 3½        |    |
| Fluid catalytic cracked                  | None                        | 13                           | 11                             | 6 weeks                              | 4         |    |
| Do                                       | 0.01                        | 3                            | 5                              | None at 12 weeks                     | 3½ 20     |    |

These results show this copolymer is highly effective in inhibiting the formation of residue and is also somewhat effective in stabilizing the color of the oils.

For purposes of comparison with the above, samples of a catalytic cracked No. 2 fuel oil were treated with 0.045 wt. percent of several different dispersing agents that are commonly employed as lubricating oil detergents. The samples were subjected to the aging test described above. After two months' storage in the dark at 110° F. in vented bottles all samples contained as much or more precipitate than the untreated control sample. The dispersing agents tested are listed in Table VIII.

Table VIII

| Dispersing Agent                          | Condition of Oil Sample After 2 Months' Storage At 110° F. in Vented Bottles |
|-------------------------------------------|------------------------------------------------------------------------------|
| None (control sample)                     | Light ppt.                                                                   |
| Barium Petroleum Sulfonate                | More ppt. than control.                                                      |
| Cobalt Petroleum Sulfonate                | Much more ppt. than control.                                                 |
| Sodium Petroleum Sulfonate                | More ppt. than control.                                                      |
| Octadecylidimethylamine+triethylphosphite | Ppt. equal to control.                                                       |
| Triethylene tetramine+naphthenic acid     | Sl. more ppt. than control.                                                  |
| Polybutene #16-Alkylated Barium Phenolate | More ppt. than control.                                                      |
| Sodium, Potassium-Alkylphenol Sulfonate   | Sl. more ppt. than control.                                                  |
| No. 40 White Oil Sulfonamide              | More ppt. than control.                                                      |
| Calcium Naphthenate                       | Do.                                                                          |
| Ethylene oxide condensation product       | Ppt. equal to control.                                                       |
| Alkylated Benzene Barium Sulfonate        | More ppt. than control.                                                      |

The negative results obtained with the above orthodox dispersing agents commonly used in lubricating oils and which might have been expected to function effectively as stabilizers in fuel oils, are in striking contrast to the results obtained using the instant copolymers as stabilizers for fuel oils.

Samples of badly deteriorated catalytic cracked fuel oil No. 2 which had been drum aged for four years in the absence of treating agents, were evaluated in a pumping test alone and together with 0.0025 wt. percent of technical lauryl methacrylate/beta-diethylaminoethyl methacrylate, 80/20, copolymer. In this test one gallon portions of the oil under examination are charged into a small reservoir which is connected by a copper piping system to a small commercial fuel oil pump and a strainer assembly so arranged that the sample of oil can be cycled indefinitely through the strainer. At the end of the cycling period, which is usually two to five days depending on the rate of plugging of the screen measured by means of a pressure gauge placed in the line just ahead of the screen, the screen is removed and the weight of solids collected on the screen is determined.

One gallon samples of the aged No. 2 fuel oil were subjected to this pumping test for 45 and 90 hours, respec-

tively. In both runs the screen was badly plugged by the insoluble residue present in the oil. When another one gallon sample of the same deteriorated oil that was treated to contain 0.0025 wt. percent of technical lauryl methacrylate/diethylaminoethyl methacrylate, 80/20, copolymer was cycled, the screen from the test assembly was practically free of deposits. The additive had prevented the insoluble residue from adhering to the screen. The quantities of residue adhering to the screen are given in Table IX.

Table IX

| Test Sample                                                                                         | Hours Cycled | Wt. of Deposit on Screen, mg. |
|-----------------------------------------------------------------------------------------------------|--------------|-------------------------------|
| Aged Fuel Oil alone                                                                                 | 45           | 155                           |
| Aged Fuel Oil alone                                                                                 | 90           | 270                           |
| Aged Fuel Oil+0.0025 wt. percent technical lauryl methacrylate/diethylaminoethyl methacrylate 80/20 | 120          | 19                            |

The advantage obtained by the use of a small amount of a conventional metal deactivator in combination with one of the herein considered copolymers in the polymerization of fuel oil is illustrated in the following test:

Samples of catalytic cracked No. 2 fuel oil distillate were inhibited by incorporating therein small amounts of technical lauryl methacrylate/diethylaminoethyl methacrylate, 80/20, copolymer and di-(2-hydroxybenzal)-1,2-propylenediamine, a conventional metal deactivator. The samples were subjected to an accelerated storage test in vented glass bottles at 110° F. for 12 weeks in the dark. At the end of the 12 weeks' aging period the samples were analyzed for soluble and insoluble residue using the procedure described in Example B. The results of the tests are as follows:

Table X

| Fuel | Additives                                  | Residue After 12 Weeks at 110° F. |                        |
|------|--------------------------------------------|-----------------------------------|------------------------|
|      |                                            | Soluble, mg./100 cc.              | Insoluble, mg./100 cc. |
| A    | None                                       | 11                                | 7                      |
| A    | +0.02% Copolymer                           | 2                                 | 4                      |
| A    | +0.02% Copolymer+0.0005% metal deactivator | nfl                               | 2                      |
| B    | None                                       | 13                                | 11                     |
| B    | +0.02% Copolymer+0.0005% metal deactivator | 2                                 | 2                      |

It will be understood that while the foregoing examples and tables have disclosed a considerable number of specific polymers adapted for use in the compositions of the present invention, these are merely illustrative and that the present invention broadly comprises a fuel oil containing at least 0.001% by weight thereof of an oil-soluble, basic amino nitrogen-containing addition-type polymer of a plurality of polymerizable ethylenically unsaturated compounds at least one of which is amine-free and at least one of which contains at least 8 carbon atoms, the polymer containing 0.1% to 3.5%, by weight thereof, of basic amino nitrogen.

The polymers used in the present invention are actually copolymers derived from at least two different polymerizable compounds, one of which must be amine-free, at least one of which must contain from 8 to about 18 carbon atoms in an aliphatic hydrocarbon chain which in the polymer is not part of the main polymer chain, thereby providing an oleophilic structure, and at least one of which must contain a basic amino nitrogen structure, and the copolymers must contain at least 0.1% but not more than 3.5%, by weight thereof, of basic amino nitrogen, preferably between 0.2% and 3.0%. The polymer can be derived from not only two different polymerizable compounds as above but also from one or more additional polymerizable compounds that do not by themselves form

oil-soluble polymers, providing the proportions are restricted to insure that the polymers have the requisite oil solubility and that no substantial change in the valuable properties of these polymers as sludge inhibitors and dispersants. A basic requirement is that the copolymer formed must have at least a limited solubility in the fuel oil, i. e., at least 0.001% by weight. The term "oil-soluble" is used herein to denote a solubility of at least 0.001%, by weight, of the polymer in the fuel oil.

As the oleophilic components of copolymers useful in the preparation of the improved fuel oil compositions of this invention there can be employed polymerizable esters, amides, ethers, and hydrocarbons characterized by the presence of at least 8 carbon atoms, preferably with 6 or more in a straight chain, and at least one carbon-carbon double bond capable of participation in free radical initiated addition copolymerization reactions. Examples of oleophilic components that come within the purview of this invention are: saturated and unsaturated long-chain esters of unsaturated carboxylic acids such as decyl acrylate, 3,5,5-trimethylhexyl methacrylate, 9-octadecenyl methacrylate; unsaturated esters of long-chain carboxylic acids such as vinyl stearate; long-chain esters of vinylene dicarboxylic acids such as methyl lauryl fumarate; N-long-chain hydrocarbon substituted amides of unsaturated acids such as N-octadecyl acrylamide; long-chain monoolefins such as the alkyl or acyl substituted styrenes, e. g., dodecylstyrene, and the like. Obviously, these components can be employed alone or in various combinations and, in general, make up the majority of the polymeric additive in order to insure proper oleophilic character. The technical lauryl methacrylate obtained from the commercial mixture of long-chain alcohols in the C<sub>10</sub> to C<sub>18</sub> range derived from coconut oil is an especially useful oleophilic component of the copolymer but the group of acrylic and alkacrylic esters of aliphatic alcohols of at least 8 carbons are, in general, well suited as the oleophilic component of the copolymer.

The basic amino nitrogen-containing component that imparts sludge inhibiting and dispersant properties to the polymers useful in this invention, can be introduced through the use of appropriate copolymerizable monomers containing primary, secondary or tertiary amino nitrogen that is attached ultimately to the chain of the polymer as part of an extralinear substituent group in which the nitrogen is joined extranuclearly only to non-benzenoid carbon atoms. There can be employed in the copolymerization monomers such as glycidyl acrylate or vinyl chloroacetate which introduce groups reactive toward ammonia or amines and thus provide a means of attaching the necessary basic amino groups to the polymer chain. Attachment of the amino groups to the main copolymer carbon chain can be through strictly hydrocarbon structures or through ether, ester, or amide linkages.

Particular examples of the basic amino-containing monomers include the basic amino substituted olefins such as p-(beta-diethylaminoethyl)styrene; basic nitrogen-containing heterocycles carrying a polymerizable ethylenically unsaturated substituent, e. g., the vinyl pyridines and the vinyl alkyl pyridines such as 2-vinyl-5-ethyl pyridine; esters of basic amino alcohols with unsaturated carboxylic acids such as the alkyl and cycloalkyl substituted aminoalkyl and cycloalkyl esters of the acrylic and alkacrylic acids, e. g., beta-methylaminoethyl acrylate, 4-diethylaminocyclohexyl methacrylate, beta-beta-didodecylaminoethyl acrylate, and the like, unsaturated ethers of basic amino alcohols such as the vinyl ethers of such alcohols, e. g., beta-aminoethyl vinyl ether, beta-diethylaminoethyl vinyl ether, and the like; amides of unsaturated carboxylic acids wherein a basic amino substituent is carried on the amide nitrogen such as N-(beta-dimethylaminoethyl)-acrylamide; polymerizable unsaturated basic amines, e. g., diallylamine, and the like. In this specification and claims the term "basic amino nitrogen" is used in the generic

sense to cover the primary, secondary and tertiary amine including, as stated above, the basic nitrogen-containing heterocycles.

Because of their relatively greater basicity and more effective sludge suspending and inhibiting properties, the polymerizable ethylenically unsaturated compounds containing a basic tertiary amino group are preferred and those having only primary basic amino groups are least desirable. Particularly outstanding and readily available basic amino nitrogen-containing components are the alkyl and cycloalkyl substituted tertiary aminoalkyl and cycloalkyl esters of acrylic and alkacrylic acids.

The basic amino nitrogen-containing component of the copolymer must be present in a minor proportion by weight corresponding to no more than 3.5% and no less than 0.1% of basic amino nitrogen by weight of the polymer. Above the higher level, which, for example, corresponds to about 50% by weight of amino monomer in a lauryl methacrylate/beta-diethylaminoethyl methacrylate copolymer, and at less than the lower level, the performance of the polymer as a sludge inhibitor falls off rapidly. It is preferred that the basic amino nitrogen content be within the range of 0.2% to 3.0% by weight of the polymer.

While the polymers as herein defined are highly effective as fuel oil stabilizers, homopolymers of aminoethyl methacrylates, preferred components of the copolymers used in this invention, are without effect on the formation of sediment in fuel oils. Even when they contain long hydrocarbon chains they are ineffective and actually accelerate formation of sediment in some instances.

Table XI shows the effect of various aminoethyl methacrylate homopolymers in the test used with respect to Table I.

Table XI  
HOMOPOLYMERS OF BASIC MONOMERS

| 40                                                     | Homopolymer | Concen-<br>tration | Days to first<br>appearance of— |          |
|--------------------------------------------------------|-------------|--------------------|---------------------------------|----------|
|                                                        |             |                    | Haze                            | Sediment |
| 1. Control                                             |             |                    | 4                               | 7        |
| 2. Beta (N, N-dibutylamino) ethyl methacrylate         |             | .005               | 4                               | 5        |
| 45 3. Beta (N-tertiarycetylamino) ethyl methacrylate   |             | .10                | 5                               | 5        |
| 4. Beta (N, N-di-2-ethylhexylamino) ethyl methacrylate |             | .005               | 3                               | 3        |
| 5. Beta (N, N-diethylamino) ethyl methacrylate         |             | .05                | 5                               | 5        |
| 6. Beta (N, N-diethylamino) ethyl methacrylate         |             | .005               | 2                               | 3        |
| 50                                                     |             | .10                | 3                               | 3        |
|                                                        |             | .005               | 3                               | 3        |

The sludge-inhibiting and dispersing polymers used in this invention can contain limited amounts of copolymerizable components that do not necessarily contribute either to improve solubility or inhibiting and dispersing action but merely serve as fillers or extenders for the active components. Typical examples of these filler components include the well-known shorter chain ethylenically unsaturated polymerizable monomers such as the vinyl and allyl formates, acetates, propionates, butyrates, and the like; polymerizable unsaturated short-chain hydrocarbons, e. g., the monoolefins such as ethylene, propylene, isobutylene, styrene, vinyltoluene, and the like, and the short-chain dienes such as 1,3-butadiene, isoprene, and the like; unsaturated short-chain carboxylic acids and their derivatives such as the alpha-methylene carboxylic acids and their derivatives, e. g., acrylic acid, methyl methacrylate, acrylonitrile, methacrylamide, and the like; the short-chain unsaturated ethers, particularly the vinyl and allyl ethers, e. g., ethyl vinyl ether, butyl vinyl ether, allyl glycidyl ether, and the like. These and other familiar monomers that are available at moderate cost, can be employed for this purpose in proportions ranging up to as much as 79%, by weight, in representative polymers although it is preferred they should not exceed 65% by weight of the polymer.

## 13

In addition, inclusion of minor proportions of N-hydrocarbon-substituted amides of unsaturated carboxylic acids will be found beneficial. Especially suitable as polymerizable components of the polymer are the N-hydrocarbon-substituted acrylamides including N-tertiary-butylacrylamide, N-tertiary-octylacrylamide, and, particularly, the N-arylacrylamides such as methacrylanilide and acrylanilide.

The polymers employed in the improved fuel oil compositions of this invention can be represented by the following schematic formula:



wherein M is the structural unit joining the various substituent groups to the main chain of the polymer; R<sub>o</sub> is the required oleophilic structure, R<sub>e</sub> is the basic amino containing structure that imparts sludge dispersency, and R<sub>e</sub> is the optional extender structure; and x, y and z represent the proportions of these various structures in the polymer. M can be an ether, ester or amide group and n is a cardinal number no greater than 1; i.e., 0 or 1; R<sub>o</sub> is a straight or branched chain hydrocarbon radical of from 8 to 18 carbon atoms, R<sub>e</sub> is a monovalent organic radical free of reactive hydrogen and is preferably a solely hydrocarbon radical of less than 8 carbon atoms and when n is 0, R<sub>e</sub> can be hydrogen; and R<sub>e</sub> is a primary, secondary, or tertiary amino radical of the structure



in which the nitrogen is bonded extra nuclearily only to hydrogen or aliphatic carbon and in which A is a hydrocarbon radical of 1-18, preferably 2 to 6 carbon atoms, B and D are hydrogen or hydrocarbon radicals of no more than about 18 and, preferably, no more than 6, carbon atoms, and B or D can be joined with A to form heterocycle. The proportions of the various structures in the polymer, as represented by x, y and z in the schematic formula, normally will be in the range; x from 20% to 99%; y from 0.5% but, preferably from 1% to 50%; and z from 0% up to 79% but, preferably, only up to 65%, all percentages being by total weight of the polymer. Within these ranges, optimum proportions will be determined both by the properties contributed to the polymer by the individual polymerizable components going into its composition and the particular properties of the polymer which it is desired to emphasize.

The concentration of the copolymer in the fuel oil will vary to some extent depending on the effectiveness of the particular copolymer, the particular fuel oil, and the degree of stability required. Generally, a concentration of at least 0.001% by weight of the fuel oil, will be used and a concentration of 0.1% will not be normally exceeded except where master batches containing 50% or more of the copolymer, by weight of the oil, are made up for convenience in processing and shipping prior to dilution of the oil. Concentrations of between 0.002% and 0.01%, by weight of the fuel oil, are usually adequate.

The copolymers may be incorporated and used in the fuel oil together with conventional antioxidants and metal deactivators as illustrated in Table X, such additives sometimes being employed to impart other desirable characteristics to the oil.

The present invention is applicable in the stabilization of any fuel oil which upon storage normally tends to undergo deterioration. It is particularly useful in the stabilization of fuel oils entirely composed of catalytic cracked oil or containing a substantial proportion of catalytic cracked oil, e.g., at least 20%, by weight thereof, inasmuch as the catalytic cracked fuel oils are notoriously subject to deterioration on storage.

An advantage of this invention is that it provides an

75

## 14

economical and practical means of effectively stabilizing fuel oils. An outstanding advantage is that it provides a means for the production of catalytically cracked fuel oils with greatly improved resistance to sludge and gum formation on storage and, to some extent of improved color stability.

A still further advantage of this invention is that the polymers used also have rust-inhibiting properties. To illustrate, a 80/20 copolymer of technical lauryl methacrylate and diethylaminoethyl methacrylate was dissolved in a cracked fuel oil distillate to a concentration of 0.0025% by weight. The solution was then stored in a inverted clear glass bottle exposed to indirect sunlight at room temperature; the bottle containing water in its lower third. A strip of mild steel was inserted so as to extend through the water, oil, and air phases in the bottle. This is an accelerated test for the rusting which occurs when a fuel oil containing water is stored in a steel container. For comparison, an untreated oil and an oil containing a commercial rust inhibitor were similarly stored. After two days, the steel strip in the latter two cases showed rusting in the water phase but in the case of the oil containing the dissolved polymer, no rusting took place at any point on the steel strip during storage for seven days.

As many apparently widely different embodiments of this invention may be made without departing from the spirit and scope thereof, it is to be understood that the invention is not limited to the specific embodiments thereof except as defined in the appended claims.

The invention claimed is:

1. A petroleum base fuel oil containing as a sludge inhibiting and dispersing agent at least 0.001% by weight of an oil soluble, basic amino nitrogen-containing addition type copolymer containing in combined form as its essential monomeric components copolymerizable ethylenically unsaturated compounds each containing only one polymerizable ethylenic linkage, at least one of which component is amine-free and contains from 8 to about 18 carbon atoms in an aliphatic hydrocarbon chain which in the polymer is not part of the main chain, and one of the components as it exists in the polymer containing a basic amino nitrogen in the side chain, said copolymer containing 0.1% to 3.5% by weight of basic amino nitrogen and said copolymer having an inherent viscosity of 0.1 to 3.0 as determined at 0.1% weight-volume concentration in benzene at 25° C.
2. A fuel oil composition as set forth in claim 1 wherein said fuel oil comprises at least about 20%, by weight thereof, of catalytic cracked oil.
3. A fuel oil composition as set forth in claim 2 wherein said oil-soluble polymer is present in a proportion of 0.002% to 0.01% by weight of said fuel oil.
4. A fuel oil composition as set forth in claim 1 wherein said oil-soluble polymer is present in a proportion of 0.002% to 0.01% by weight of said fuel oil, has an inherent viscosity of 0.2 to 1.0 as determined at 0.1% weight/volume concentration in benzene at 25° C., and contains 0.2% to 3.0%, by weight thereof, of basic amino nitrogen.
5. A petroleum base fuel oil containing as a sludge inhibiting and dispersing agent at least 0.001% by weight of an oil soluble, basic amino nitrogen-containing addition type copolymer containing in combined form as its essential monomeric components copolymerizable ethylenically unsaturated compounds, one of which is from the group consisting of acrylic and alkacrylic esters of aliphatic alcohols of from 8 to about 18 carbon atoms and one of the components containing a basic tertiary amino group in the side chain, said copolymer containing 0.1% to 3.5% by weight of basic amino nitrogen and said copolymer having an inherent viscosity of 0.1 to 3.0 as determined at 0.1% weight/volume concentration in benzene at 25° C.
6. A fuel oil composition as set forth in claim 5

## 15

wherein said oil-soluble polymer is present in a proportion of 0.002% to 0.01% by weight of said fuel oil, has an inherent viscosity of 0.2 to 1.0 as determined at 0.1% weight/volume concentration in benzene at 25° C., and contains 0.2% to 3.0%, by weight thereof, of basic amino nitrogen.

7. A petroleum base fuel oil containing as a sludge inhibiting and dispersing agent at least 0.001% by weight of an oil soluble, basic amino nitrogen-containing addition type copolymer containing in combined form as its essential monomeric components copolymerizable ethylenically unsaturated compounds, one of which is from the group consisting of acrylic and alkacrylic esters of aliphatic alcohols of from 8 to about 18 carbon atoms and one of the components is from the group consisting of alkyl and cycloalkyl substituted tertiary aminoalkyl and amino cycloalkyl esters of acrylic and alkacrylic acids, said copolymer containing 0.1% to 3.5% by weight of basic amino nitrogen and said polymer having an inherent viscosity of 0.1 to 3.0 as determined at 0.1% weight/volume concentration in benzene at 25° C.

8. A fuel oil composition as set forth in claim 7 wherein in said oil-soluble polymer is present in a proportion of 0.002% to 0.01% by weight of said fuel oil, has an inherent viscosity of 0.2 to 1.0 as determined at 0.1% weight/volume concentration in benzene at 25° C., and contains 0.2% to 3.0%, by weight thereof, of basic amino nitrogen.

9. A petroleum base fuel oil containing as a sludge inhibiting and dispersing agent at least 0.001% by weight of an oil soluble, basic amino nitrogen-containing addition type copolymer containing in combined form as its essential monomeric components copolymerizable ethylenically unsaturated compounds, one of which is from the group consisting of acrylic and alkacrylic esters 35

## 16

of aliphatic alcohols of from 8 to about 18 carbon atoms and one of the components is beta-diethylaminoethyl methacrylate, said copolymer containing 0.1% to 3.5% by weight of basic amino nitrogen and said polymer having an inherent viscosity of 0.1 to 3.0 as determined at 0.1% weight/volume concentration in benzene at 25° C.

10. A petroleum base fuel oil containing as a sludge inhibiting and dispersing agent from 0.002% to 0.01% by weight of an oil soluble, basic amino nitrogen-containing addition type copolymer containing in combined form as its essential monomeric components copolymerizable ethylenically unsaturated compounds, one of which is lauryl methacrylate and one of which is beta-diethylaminoethyl methacrylate, said copolymer containing 0.1% to 3.5% by weight of basic amino nitrogen and said copolymer having an inherent viscosity of 0.1 to 3.0 as determined at 0.1% weight/volume concentration in benzene at 25° C.

11. A petroleum base fuel oil as set forth in claim 1, 20 containing from 0.1% to about 50% by weight of the oil soluble, basic amino nitrogen-containing addition type copolymer.

## References Cited in the file of this patent

## UNITED STATES PATENTS

|           |                 |       |               |
|-----------|-----------------|-------|---------------|
| 2,138,763 | Graves          | ----- | Nov. 29, 1938 |
| 2,311,548 | Jacobson et al. | ----- | Feb. 16, 1943 |
| 2,448,542 | McQueen et al.  | ----- | Sept. 7, 1948 |
| 2,666,044 | Catlin          | ----- | Jan. 12, 1954 |

## OTHER REFERENCES

Petroleum Engineer, November 1950, pages C-31 and C-32.